

## UNITED STATES PATENT OFFICE

2,135,363

## SOLVENT REFINING OF MINERAL OIL

René de M. Taveau, Beacon, Louis A. Clarke, Fishkill, and Robert E. Manley, Beacon, N. Y., assignors to The Texas Company, New York, N. Y., a corporation of Delaware

No Drawing. Application July 5, 1934,  
Serial No. 733,864

2 Claims. (Cl. 196—13)

This invention relates to refining mineral oil with solvents for the production of lubricating oils.

The invention contemplates the production of lubricating oil from mixed base crudes and the like containing asphaltic, naphthenic and paraffinic constituents, including wax, by a process involving treatment of the oil with a solvent adapted to separate and remove the asphaltic bodies, extraction of the de-asphaltized oil with a solvent adapted to separate and remove the naphthenic constituents of low lubricating value, and thereafter dewaxing this refined oil.

The invention contemplates carrying out the successive steps for the removal of asphaltic and naphthenic bodies from the oil through the medium of a common solvent in conjunction with a suitable extraction solvent of the character of furfural. A common solvent suitable for this purpose is one which is adapted to precipitate the asphaltic constituents while maintaining the remaining oil in solution, and which is also adapted to serve as a diluent during the subsequent extraction and, if desired, dewaxing step. We have found that a suitable solvent for this purpose comprises a solvent selected from the group of aliphatic alcohols containing up to seven carbon atoms, their isomers, mixtures thereof, including mixtures of the isomers with the normal alcohols.

The invention therefore comprises mixing oil containing asphaltic, naphthenic and paraffinic constituents with an aliphatic alcohol, or a mixture of aliphatic alcohols of the above character in sufficient proportion to precipitate all or a substantial portion of the asphaltic constituents while retaining the remaining oil in solution. The precipitated asphaltic constituents are then removed from the dilute mixture, following which the dilute mixture is subjected to extraction with an extractive solvent of the character of furfural. Other extractive solvents, such as acetone, nitro benzene, etc., may be employed instead of furfural, although furfural is preferred since a mixture of aliphatic alcohol with furfural provides a very effective mixture for extracting mixed base oils to separate therefrom a maximum yield of oil having the desired lubricating qualities.

We are aware that certain of the aliphatic alcohols have been employed in the prior art heretofore for the purpose of removing asphaltic constituents from mineral oil. It is novel, however, to employ such alcohols in conjunction with an extractive solvent of the character of furfural for the purpose of practicing our invention.

We have found it advantageous to remove the asphaltic constituents from oil prior to extraction with furfural. Furfural tends to extract the naphthenic constituents from the oil in preference to the asphaltic bodies and consequently, in the case of certain oils which are rich in asphaltic material, the oil, after extraction with furfural, may still contain substantial amounts of undesirable asphaltic matter. The presence of this asphaltic matter, however, tends to interfere with the desired selective action of the furfural. Consequently, by removing the asphaltic bodies from the oil prior to extraction with furfural, the latter solvent is used to greater effect so that the naphthenic bodies can be more efficiently extracted from the oil. Accordingly, the combination of alcohol treatment for the removal of asphaltic bodies, followed by furfural extraction to remove the naphthenic constituents, provides a suitable method for refining heavy residual oils derived from mixed base crudes, and which contain substantial amounts of asphaltic material.

Furthermore, the presence of the alcohol in the oil during subsequent extraction with furfural serves to bring about a more effective and intimate contact between the furfural and the oil, due to the diluent effect on the oil.

In the case of certain types of oil, aliphatic alcohols possess certain desirable modifying effects upon the selective action of furfural. For example, certain highly paraffinic oils such as may be derived from Pennsylvania Crude are relatively insoluble in furfural, and the undesirable constituents of low lubricating value may be difficult of removal. Amyl alcohol if present in suitable proportions with the furfural serves as a pro-solvent thereby tending to increase the solubility effect of furfural for the oil constituents of low lubricating value and thus facilitating their removal in the extract layer.

On the other hand with certain other types of oil furfural possesses certain desirable modifying effects upon the deasphaltizing action of aliphatic alcohols. For example, certain oils such as Mid-Continent Residuum are difficult to deasphaltize because of the relatively high solubility of the asphaltic constituents in amyl alcohol. Furfural if present in suitable proportions with the alcohol serves as an anti-solvent thereby tending to decrease the solubility effect of the alcohol for the asphaltic constituents, and thus facilitate their removal in the insoluble asphaltic layer.

Lubricating oil as prepared by subjecting crude

oil to distillation, contains constituents of intermediate lubricating value. When extracting the oil with furfural alone, these constituents may be removed in the extract layer due to their solubility in the furfural. However, when extracting with furfural in the presence of alcohol, due to the favorable solvent effect of the alcohol on such constituents, they are removed in the raffinate layer and thereby enhance the quality of 10 raffinate.

Our invention is adapted to the treatment of wax-bearing oil when employing certain of the aliphatic alcohols as, for example, amyl alcohol as the common solvent. Since amyl alcohol, under certain conditions of temperature and dilution, may tend to precipitate some of the waxy constituents, the latter will be precipitated along with the asphaltic bodies and thus decrease the amount of wax to be removed in the subsequent 20 treatment of the oil.

However, when treating wax-bearing oil containing substantial amounts of wax, the raffinate may contain substantial proportions of the wax. In that case dewaxing may be readily effected 25 since the mixture is already in a dilute condition and contains substantial amounts of furfural or extraction solvent which, in itself, provides an anti-solvent for the wax. If desired, additional qualities of diluent and anti-solvent may be added 30 thereto to further facilitate the removal of wax, which may be accomplished by the usual mechanical means involving filtration, centrifuging and cold settling.

An important advantage of our invention resides 35 in effecting the removal of asphaltic and naphthenic bodies prior to dewaxing since, in many instances, these bodies or the colloidal substances associated therewith, tend to inhibit complete separation between oil and wax. The presence 40 of these materials also impedes removal of the separated wax from the oil, particularly in the case of dewaxing by filtration.

In the practice of our invention for the treatment of a heavy residual cylinder stock fraction 45 derived from mixed base crudes, the oil may be mixed in a ratio of about one volume of oil to four or five volumes of alcohol. The alcohol comprises preferably butyl alcohol, amyl alcohol or a mixture of butyl and isopropyl alcohol. The 50 mixture is maintained at a temperature of about 120° F. or 150° F. or at a temperature high enough to keep the wax in solution. Sufficient pressure is employed to maintain the alcohol in a liquid state at the temperatures employed.

The temperature selected, as well as the proportion 55 of the alcohol, will depend upon the nature of the oil undergoing treatment. If the temperature is too high, a substantial amount of the asphalt may remain dissolved in the oil. On the other hand, if the temperature is too low 60 substantial amounts of oil may be separated along with the asphalt.

The treatment with alcohol may be effected in batch or by countercurrent operation. The asphaltic material may be separated from the mixture of oil and alcohol by settling or centrifuging. We have found that centrifuging proves a very effective method of removing the precipitated asphaltic bodies. If desired the mixture may be 70 subjected to settling into layers and the asphaltic layer then subjected to settling.

After removal of the insoluble asphaltic constituents, all or part of the alcohol may be stripped from the resulting de-asphaltized oil. 75 For example, sufficient of the alcohol may be

removed to leave a mixture containing about one part of alcohol to two parts of oil. To this mixture furfural is added to form a mixture of two parts of furfural to one part of oil. This mixture is then maintained preferably at a temperature of 120° F. to 225° F. to effect separation into layers respectively rich in paraffinic and naphthenic constituents.

The presence of the alcohol in the mixture serves to facilitate extraction with furfural since 10 it acts as a modifying solvent and diluent. By virtue of its diluent effect, it permits more effective contact between furfural and oil and also more rapid settling and separation into layers.

The extraction with furfural may also be carried out in either batch or countercurrent operation.

Where the oil undergoing treatment contains wax, the resulting raffinate or paraffinic fraction will contain substantial amounts of wax and it is therefore necessary to subject the mixture to dewaxing. To facilitate dewaxing, further quantities of alcohol may be added, if necessary, in order to increase the extent of dilution. The mixture already contains some furfural which 25 serves as a wax anti-solvent. Additional quantities of wax anti-solvent liquid may be added, if desired.

The resulting mixture is then chilled to temperatures of the order of -10° F. whereupon the 30 wax is solidified. The cold mixture may then be centrifuged, filtered or settled in order to separate and remove the wax. Where it is filtered it may advantageously be filtered in the presence of a suitable filter-aid material such as Filter Cel, 35 fuller's earth, diatomaceous earth, or the like.

The solvents contained in the filtrate and wax may be removed by distillation or in any other suitable manner and recovered for reuse.

The invention is not restricted to the particular 40 operating conditions mentioned above. The temperatures as well as the solvent proportions set forth may be varied depending on the nature of the oil undergoing treatment.

The invention is not limited to the treatment 45 of residual lubricating oil fractions, as above described, but is also adapted to the treatment of distillate lubricating fractions.

Obviously many modifications and variations 50 of the invention, as hereinbefore set forth, may be made without departing from the spirit and scope thereof, and therefore only such limitations should be imposed as are indicated in the appended claims.

We claim:

1. In the refining of heavy residual wax-bearing mineral lubricating oil stock derived from Mid-Continent crude, the method comprising mixing the oil with a mixture of isopropyl alcohol, butyl alcohol and furfural in an amount sufficient to precipitate asphaltic constituents of oil while retaining remaining constituents of the oil in solution, removing the asphaltic constituents from the mixture of oil and solvent, extracting the mixture of oil and solvent with a further quantity of furfural, forming an extract phase containing low viscosity index constituents of a raffinate phase containing high viscosity index constituents and wax, mixing additional furfural and alcohol with the raffinate phase 70 such that the solvent mixture has selective action as between oil and wax, chilling the mixture to a temperature of around 0° F. and below to precipitate wax, and removing the wax so precipitated.

2. The method of removing asphalt from heavy residual wax-bearing oil at a temperature in the range 120° to 150° F. and substantially above the temperature at which waxy constituents of the oil become solid which comprises subjecting the oil to countercurrent contact with a substantially non-aqueous mixture of isopropyl alcohol, butyl alcohol and extraction solvent having the essential selective action of furfural as between naphthenic and paraffinic constituents of oil in proportion such that the alcoholic mixture has substantially no solvent action on the asphaltic constituents and substantially complete solvent action on the non-asphaltic constituents of the oil, forming an asphaltic phase comprising asphaltic constituents mixed with a small amount

of solvent, and a non-asphaltic phase comprising non-asphaltic constituents dissolved in the bulk of the solvent, separating the two phases, extracting the non-asphaltic phase with a further quantity of extraction solvent to remove low viscosity index constituents thereby producing a raffinate phase of high viscosity index containing wax, and dewaxing the raffinate phase in the presence of the extraction solvent and a further quantity of alcohol such that the solvent mixture has selective action as between oil and wax at the dewaxing temperature. 5 10

RENÉ DE M. TAVEAU.

LOUIS A. CLARKE.

ROBERT E. MANLEY.

15